

# UNITED STATES PATENT OFFICE.

SAMUEL WEIN, OF NEW YORK, N. Y., ASSIGNOR TO JEROME A. STRAUSS, TRUSTEE.

## METAL ALLOY.

1,102,618.

Specification of Letters Patent.

Patented July 7, 1914.

No Drawing.

Application filed October 6, 1913. Serial No. 793,499.

To all whom it may concern:

Be it known that I, SAMUEL WEIN, a subject of the Emperor of Austria-Hungary, and a resident of New York, in the county 5 of New York and State of New York, have invented certain new and useful Improvements in Metal Alloys, of which the following is a specification.

This invention relates to metallic alloys, 10 particularly alloys of aluminum.

In making mechanical parts in the industrial arts in situations where weight must be reduced to a minimum aluminum has usually been employed as the lightest of 15 all metals. However, owing to the low tensile strength of this metal, the advantage of its low specific gravity is in many cases offset where strength as well as lightness in weight is required. Many attempts have, 20 therefore, been made to secure an alloy with aluminum as a base which shall combine the lightness of aluminum with the higher tensile strength of the heavier metals. One of the most common as well as the best alloy 25 of aluminum hitherto used has been the alloy of aluminum and zinc with or without some other metal, as copper or the like. This alloy, while giving some measure of satisfaction in certain cases, is not entirely 30 satisfactory, for the reason that, when the proportion of zinc is increased to give higher tensile strength, the alloy is rendered brittle, and is thus unable to withstand shocks and jars as encountered in many im- 35 portant mechanisms in which the alloy is to be used. Also, difficulty has been experienced in obtaining uniform castings. Very frequently one pot of metal properly alloyed, fluxed, and stirred, cleaned, and 40 skinned, drawn under a pyrometer, poured into two similar molds side by side at the same heat and time, will give two widely different results in strength determinations from test bars in the two molds. Very fre- 45 quently blow holes are found in the castings which are very difficult to account for, in view of the extreme care which has been exercised in preparing and casting the metal.

The object of the present invention is to 50 overcome these difficulties, so as to secure an alloy of aluminum which combines the low specific gravity of the latter with high tensile strength, toughness, freedom from oxidation to any appreciable extent in the at-

mosphere, and various other advantageous properties which will more fully herein-after appear.

I have discovered that by adding a combining agent which enters into combination with the aluminum and zinc I am enabled to produce an aluminum-zinc alloy which combines all of the advantageous properties above set forth without the defects. This combining agent is the metal tellurium in small proportion to the aluminum and zinc, preferably from  $\frac{1}{4}$  to 1%. In making the alloy the aluminum is first preferably melted, then the proper proportion of zinc is added until the two are fused together to a homogeneous mass. The tellurium is then inserted into the mixture, preferably with suitable tongs, or other instrument, to deposit the same at the bottom of the crucible and permit the same to transfuse through the entire body of metal. The proportion of the various metals may be varied, the aluminum varying from 50 to 85 parts, the zinc from 49 down to 14 parts, and the tellurium from  $\frac{1}{4}$  to 1 part. The various proportions are to secure various degrees of hardness and toughness of the alloy, depending upon the character of its use. The tensile strength may run up as high as 48,000 pounds per square inch, and the torsional strength as high as 60,000 pounds per square inch.

The improved alloy may be rolled into sheets and drawn into wire, and when suitably annealed may be rendered sufficiently tough to be bent back on itself without fracturing. Castings as well as forgings may be made with equal ease, the metal flowing freely when cast hot or when subjected to pressure or impact when cold. The alloy is readily soldered, and a joint may be obtained which is as strong or stronger than the body of the metal. A beautiful polish may be imparted to the surface of the alloy, and the same may be left for a long time in the atmosphere without substantial oxidation. It is suitable for electrical purposes, as it has a high electrical conductivity.

Having thus described my invention, I claim as new and desire to secure by Letters Patent:

1. An alloy consisting of aluminum, zinc and tellurium.
2. An alloy comprising aluminum, zinc

and tellurium in the following proportions:—aluminum, 50 to 85% and tellurium  $\frac{1}{4}\%$  to 1%, the difference between the sum of these percentages and 100% consisting of zinc.

Signed at New York in the county of

New York and State of New York this  
fourth day of October A. D. 1913.

SAMUEL WEIN.

Witnesses:

Wm. I. COHEN,  
EVE AXEL.